

Sept. 8, 1936.

F. X. GOVERS

2,054,052

## SOLVENT REFINING OF HYDROCARBON OIL

Filed March 2, 1935



*Francis X. Govers*  
INVENTOR

BY R. J. Dearborn.

his ATTORNEY

## UNITED STATES PATENT OFFICE

2,054,052

## SOLVENT REFINING OF HYDROCARBON OIL

Francis X. Govers, Vincennes, Ind., assignor to  
 Indian Refining Company, a corporation of  
 Maine

Application March 2, 1935, Serial No. 9,005

13 Claims. (CL 196—17)

This invention relates to the treatment of hydrocarbon oil, and particularly to a method of treating mineral oil with selective solvents.

The invention broadly contemplates a process for solvent refining mineral oil for the production of lubricating oil of high viscosity index, low pour test, and other desired properties and characteristics.

The invention comprises extractively treating mineral oil stock with a selective solvent, such as furfural, for example, wherein the oil is separated into an extract phase containing low viscosity index constituents of the oil, and a raffinate phase comprising high viscosity index constituents of the oil. The two resulting phases are separately cooled, to effect alteration of mutual solubility of component parts, and centrifuged or settled to remove the component parts not retained in solution. The matter thus removed from each phase is returned, all or in part, to the zone of extraction wherein it is brought into contact with fresh oil undergoing treatment.

In the treatment of wax-bearing oil, the raffinate phase, containing substantially all of the paraffin constituents of the oil, is dewaxed, as will be more fully described, by means of selective dewaxing solvents to produce therefrom a lubricating oil of low pour test and high viscosity index.

30 In the solvent treatment of mineral lubricating oil stock with furfural, solvent action increases with elevated temperatures, and the selectivity increases with lower temperatures; thus, at 250° F. the total solvent power of the furfural is far greater than at 80° F. but the selectivity is greater at 80° F. than at 250° F. Economy, based alone on the amount of solvent used, predicates the use of high temperature, and economy based on percentage yields of high viscosity index oils 40 predicates the use of low temperatures.

I have discovered that furfural is quite selective, even at high temperatures, when saturation points for any particular constituent or component part of the mineral oil stock are not exceeded.

45 I have discovered that by the proper use of limited amounts of furfural at high temperatures, extraction refining can be practiced economically in such a way as to effect maximum action of solvent refining with minimum loss of desirable constituents while at the same time increasing the susceptibility of the raffinate phase to the refining action of certain solvents for still further improvement in color, viscosity index, sulphur, and Conradsen carbon.

I have discovered that the oils separated from the cooled extract phase are more susceptible to solvent refining than the original stock.

I have discovered that the raffinate phase, when cooled and separated from the retained extract phase, is highly susceptible to the solvent refining action of ketones, such as methyl ethyl ketone and methyl isobutyl ketone.

I have discovered that this process, when practiced in the order of the steps herein disclosed, 10 will, from any given wax-bearing lubricating stock, give higher percentage yields of low pour test oils of any given viscosity index with resultant lighter specific gravity, lower Conradsen carbon, lower sulphur, and better color, without 15 treatment with mineral acid, than any solvent process heretofore described.

I have discovered that the process, when practiced in the order of the steps as herein disclosed, 20 is particularly advantageous in the treatment of either heavy distillates, or residual oils.

I have discovered that the raffinate can be dewaxed by means of a selective solvent comprising in part the selective washing or refining solvent used in the last step of extraction, and that 25 the final result is increased yields of low pour test, high viscosity index oils of very low Conradsen carbon and sulphur.

Accordingly, the invention comprises a process for treating wax-bearing lubricating oil stock 30 in which the oil is extracted with a solvent comprising furfural at temperatures of around 170–250° F., and the mixture separated into extract and raffinate phases respectively. The extract phase will contain low viscosity index undesirable constituents, blended with a certain amount of desirable relatively higher viscosity index constituents. The raffinate phase will comprise the relatively higher viscosity index constituents of the oil containing some of the extract phase retained or suspended therein.

The two phases are separated from each other. The raffinate phase is cooled and subjected to centrifuging or settling to separate these retained extract phase bodies. The extract phase 45 is cooled, to release from solution, and subjected to centrifuging or settling to separate part of the desirable relatively higher viscosity index constituents. The separated bodies are then returned, all or in part, to the extraction zone 50 where they are brought in contact with fresh charge.

When oil is extracted with furfural at elevated temperatures, as for example around 170–250° F., the resulting raffinate phase contains an appreci- 55

able amount of extract phase material retained therein, and likewise the extract phase also retains a substantial amount of relatively higher viscosity index oil which, at the high temperature prevailing, is soluble in the solvent. Accordingly, by cooling the raffinate phase down to a temperature below 170° F., or in the range of 130-150° F., depending upon the pour test of the oil, and upon centrifuging the thus cooled raffinate phase, a substantial portion of the retained extract phase material may be separated from the raffinate phase. Similarly, in the case of the extract phase, upon cooling for example to about 110° F. and standing at this temperature, a substantial quantity of oil separates from solution.

The extract phase material, separated from the raffinate phase in the foregoing centrifuging step, comprises furfural containing oil dissolved therein. This material may be returned to the extraction zone or be mixed with fresh charge entering the extraction zone.

It is of advantage also to return the oil separated from the cooling of the extract phase to the extraction zone. This oil is of a relatively paraffinic nature and its addition to the fresh charge has a tendency to increase the selectivity of the extraction solvent or to facilitate the separation of the oil into extract and raffinate phases, respectively rich in low viscosity index and high viscosity index constituents of the oil.

Consequently, by returning the extract phase material separated from the raffinate phase, and the oil separated from the extract phase, to the extraction zone, advantage is taken of the furfural retained therein since it is thus used in the further extraction of fresh oil. It also enables the obtaining of higher ultimate yields of high viscosity index oil since the oil constituents contained in the separated material are subjected to further separating action.

The raffinate phase, after centrifuging, will still retain some extract phase material, and this and other undesirable constituents are removed by subjecting the raffinate phase to a washing treatment with a solvent adapted to effect their removal. Such a solvent may comprise, for example, a ketone such as methyl ethyl ketone, methyl isobutyl ketone or homologs.

When the oil undergoing treatment comprises a wax-bearing oil, the subsequent dewaxing operation is effected by means of a selective solvent mixture comprising, for example, a mixture of an anti-solvent liquid of the character of an aliphatic ketone, such as acetone or methyl ethyl ketone, and a good oil solvent such as benzol or toluol. The wax anti-solvent liquid component of the dewaxing solvent mixture advantageously comprises a solvent which is also suitable by itself as a washing solvent capable of dissolving from the raffinate phase any extract phase material remaining therein.

I have found that methyl ethyl ketone, for example, is a suitable solvent for this purpose. Thus, in carrying out the process of my invention, as applied to a wax-bearing oil, the resulting raffinate phase, after cooling and centrifuging to remove extract phase material, is then subjected to washing with methyl ethyl ketone.

In this washing step, the methyl ethyl ketone dissolves any remaining extract phase material retained in the cold raffinate phase, and which may comprise furfural as well as low viscosity index oil. Other impurities in the oil, insoluble or sparingly in the furfural, as for example sul-

phur compounds and other bodies which tend to form color or to produce residual carbon, will also be removed by the washing solvent.

In washing the raffinate with the wash solvent, there results a separation into two phases. One phase will comprise the solution of wash solvent liquor, furfural, color forming matter and undesirable constituents dissolved from the raffinate phase, while the other phase will comprise the purified raffinate phase in a suspended finely divided condition. These two phases can be separated by filtration. The filter cake, comprising the washed raffinate phase will, in the case of the above wax-bearing oil, contain wax constituents and, therefore, the retained wash solvent, namely, methyl ethyl ketone, is left mixed with the washed raffinate phase to serve as a component of the subsequent dewaxing solvent mixture.

Accordingly, an additional quantity of methyl ethyl ketone, together with sufficient benzol or toluol, is added to the washed raffinate to produce a solvent mixture which has selective action as between oil and wax at temperatures of the order of 0° F. and below. This mixture is then chilled to precipitate the wax and the precipitated wax constituents removed therefrom by filtering, centrifuging, settling or other mechanical means. After removal of the solvent from the dewaxed oil, the oil is finished up, for example, by contacting with solid adsorbent material to produce a finished lubricating oil product of superior characteristics.

In order to more clearly describe the invention, reference will now be made to the accompanying flow diagram which illustrates the practice of the process of my invention as applied to the treatment of wax-bearing oil such as a wax-bearing lubricating distillate derived from Mid-Continent crude.

The wax-bearing oil to be treated is conducted from a storage tank 1 and delivered by a pump through a pipe 2 to the lower portion of the separator 3.

The separator 3 comprises a vertical, cylindrical vessel provided with agitation means 4, as shown. The separator and agitating means are advantageously of the type described in my co-pending application Ser. No. 1,331, filed January 11, 1935.

The oil may be heated to suitable temperature prior to introduction to the separator 3 in which case it is passed through a heater 5. Where it is not necessary to thus heat the oil, it may be by-passed around the heater 5, as indicated in the flow diagram.

The furfural is conducted from a tank 6 through pipe 7 to the upper portion of the separator 3. As in the case of the entering oil charge, the furfural may be heated by passage through a heater 8 prior to introduction to separator 3. The amount of heating to which the solvent and oil is subjected will depend upon the particular temperature condition which it is desired to maintain within the separator 3 and it is contemplated that all of the heat may be supplied either by heating the oil or by heating the furfural alone.

The furfural being heavier than the oil flows through the separator 3 countercurrently to a rising body of oil. Intimate contact between the oil and solvent is brought about by rotation of the agitating means 4. As a result of the contact between oil and solvent within the separator, the mixture separates into extract and raffinate phases respectively. The extract phase

being of heavier specific gravity accumulates in the bottom of the separator and is withdrawn therefrom through pipe 9 to cooler 10 wherein it is cooled to a temperature of around 110° F. 5 The resulting chilled extract phase is then conducted to a settling chamber 11 wherein, upon standing at the above temperature, paraffinic oil separates from the mixture and is drawn off to a tank 12. It is to be understood that instead 10 of settling, the cooled extract phase may, of course, be subjected to centrifuging if desired.

The remaining extract phase from which the paraffinic oil has been separated is then drawn to a tank 13 wherein it may be stored for such 15 further treatment as may be desired.

The raffinate phase formed in the separator 3, and which rises to the upper portion of the separator, is withdrawn therefrom through pipe 14 to cooler 15 wherein it is cooled to a suitable temperature above the solidifying point of the wax-bearing raffinate oil. This temperature will depend upon the proportion of wax present as well as upon the viscosity of the oil. 20

The cold raffinate phase is then delivered to a 25 centrifuge or other separating means, such as a settling chamber 16, wherein the extract phase material retained therein is separated. The thus separated extract phase material is conducted to a tank 17 for return to the separator 3, as will be 30 subsequently described.

The centrifuged raffinate phase is then mixed in a mixer 19 with about equal volume of methyl ethyl ketone drawn from a tank 18. This mixing is carried out advantageously at a temperature 35 just sufficient to complete solution of the raffinate phase in the methyl ethyl ketone.

From the mixer 19, it is passed through a chiller 20 wherein it is chilled to a temperature of around 30° F. At this temperature, the paraffinic 40 constituents of the oil, including paraffin wax, will be converted to a substantially solid form.

This cold mixture is then conducted to a filter 21 wherein the liquid is separated from the solid 45 matter. The liquid or filtrate will comprise methyl ethyl ketone containing in solution extract material dissolved from the raffinate phase, as well as other undesired impurities freely soluble in methyl ethyl ketone but sparingly soluble in 50 furfural, including sulphur compounds, color-forming, as well as residual carbon-forming bodies.

The separated liquid or filtrate is withdrawn 55 from the filter 21 and conducted to a still 22. The methyl ethyl ketone is vaporized from this liquid, and the resulting vapors cooled and condensed in a cooler 23, and from there returned to the tank 18, previously mentioned.

The residual liquid remaining in the still 22, 60 comprising furfural and oil, is withdrawn to tank 24. From this tank, it is returned to the separator 3 directly, or else first mixed with fresh charge, as will be subsequently described.

The filter cake comprising paraffinic bodies of 65 the oil, including wax, remaining in the filter 21, is withdrawn through a pipe 25 to a mixer 26. Prior to introduction to the mixer, this paraffinic oil is mixed with an additional quantity of methyl ethyl ketone, from the tank 18, and also with 70 benzol drawn from a tank 27. The methyl ethyl ketone and benzol are added in the proportions of about 40% ketone to 60% benzol, and mixed with the oil in the proportion of 3 to 4 parts of solvent mixture to 1 part of oil.

75 From the mixer 26 the oil and solvent is con-

ducted to a chiller 28 wherein it is chilled to a temperature of around -10° F. in order to precipitate the wax from the solution.

The chilled mixture is then conducted to a filter 29 wherein the precipitated wax is separated 5 as a filter cake. The filter cake is removed and the solvent recovered from the wax. The dewaxed filtrate is then delivered to a still 30 for removal of the solvent which latter may be returned for use in dewaxing further oil. 10

The dewaxed oil, free from solvent, is conducted to a contact vessel 31 where it is advantageously contacted with adsorbent clay in the presence of steam at temperatures of around 400-500° F. The contacted oil is then delivered 15 to filter 32 for removal of the solid adsorbent material therefrom. The resulting filtrate, comprising finished lubricating oil of low sulphur and low carbon residue content and high viscosity index, coupled with low pour test, is delivered to a 20 tank 33.

The separated oil of paraffinic nature accumulating in tank 12, together with the extract phase material accumulating in tank 17 and the mixture of furfural and oil in tank 24, is drawn off 25 to a pipe 34. This combined material is then delivered by a pump 35 to the pipe 2, previously referred to, and wherein it is mixed with fresh oil entering the lower portion of the separator 3. Instead of combining this material in this way, those portions accumulating in tanks 17 and 24 30 may be returned directly to the upper portion of the separator 3.

The nature and amount of oil which is separated 35 from the raffinate and extract phases in the foregoing operation may be illustrated by reference to the following data obtained in the solvent refining of a wax bearing distillate having the following characteristics:

|                                        |      |    |
|----------------------------------------|------|----|
| Gravity A. P. I.                       | 25.4 | 40 |
| Viscosity Saybolt universal at 130° F. | 143  |    |
| Viscosity Saybolt universal at 210° F. | 50   |    |
| Carbon residue                         | .16% |    |
| Viscosity index                        | 71   | 45 |

The above wax distillate was subjected to counter-current extraction with furfural in the proportion of about one part of oil to two parts of solvent. This extraction was carried out in a separating tower in which the temperature at the bottom of the tower was about 170° F. and the temperature at the top of the tower about 200° F. 50

The resulting raffinate and extract phases were 55 separately cooled to a temperature of about 130° F. When the raffinate phase was thus cooled, there resulted a separation of a lower layer of material comprising about 2% oil and 98% furfural. This lower layer was removed, and the oil and solvent separated. The oil thus obtained from this lower layer amounted to about .07% of the total raffinate oil. The solvent was also removed from the upper layer comprising raffinate oil, and the following is a tabulation of the tests on this raffinate oil of the upper layer and of the separated oil in the lower layer: 60

|                                        | Raffinate oil           | Separated oil |
|----------------------------------------|-------------------------|---------------|
| Gravity A. P. I.                       | 30.5                    | 16.8          |
| Viscosity Saybolt universal at 100° F. | 221                     |               |
| Viscosity Saybolt universal at 210° F. | 43                      |               |
| Carbon residue                         | .017                    |               |
| Viscosity index                        | .97                     |               |
| Color                                  | 90 $\frac{1}{2}$ " cell | Black         |

Similarly, when the extract phase was cooled to 130° F. there resulted a separation of oil comprising about 1.65% of the extract phase. The tests on this oil, after the solvent had been removed, were as follows:

|                                       |      |
|---------------------------------------|------|
| Gravity A. P. I.                      | 24.9 |
| Viscosity Saybolt universal at 100° F | 331  |
| Viscosity Saybolt universal at 210° F | 51   |
| Viscosity index                       | 67.5 |

10 It will be observed from the foregoing that  
the cycle oil thus separated from the extract  
phase is very similar in character to the original  
wax distillate prior to extraction and thus con-  
15 tains a substantial portion of valuable oil.

15 The process of this invention is not restricted to any specific solvent or mixture of solvents, but it is contemplated that other solvents or mixed solvents, possessing the desired selective  
20 action as between constituents of the oil of differing viscosity index or between solid or liquid constituents of the oil, may be used. While the process of my invention is particularly adapted to extraction with solvent of the character of  
25 furfural, at elevated temperatures, the process is nevertheless applicable to operations in which the oil is extracted with other solvents, such as nitrobenzene, aniline etc., since, as I have already indicated, centrifuging of the resulting extract and raffinate phases permits therefrom separation of material retained in each phase due to not having realized a clear cut separation during the extractive treatment within the separation zone.

35 The mineral oil fractions, when so treated with the above solvents, are rendered particularly susceptible to the purifying action of a wash solvent, having the solvent characteristics of methyl ethyl ketone, as many undesired impurities and constituents are thus rendered soluble in the wash solvent without affecting its selective action on the high viscosity index constituents.

40

Also, as regards the dewaxing step, solvents other than methyl ethyl ketone and benzol may be employed. For example, it has been found that methyl isobutyl ketone may be substituted for methyl ethyl ketone since this solvent not only possesses anti-solvent properties of wax, but is also adapted as a wash solvent for removal from the raffinate phase and remaining extract phase material retained therein. Either one of these solvents may be employed in conjunction with benzol or toluol, or a mixture of benzol and toluol, to provide a selective dewaxing solvent mixture.

60 The process of this invention is not limited to any particular type of hydrocarbon oil or petroleum fraction. It is adapted to the treatment of either distillate or residual fractions of petroleum, and while the invention has been described as to the separation of wax from wax-bearing lubricating oil stocks, it is contemplated that it may also be employed for the separation of oil from petrolatum or other waxy concentrates.

Moreover, it is contemplated that, as regards the specific manner in which the invention is practiced, temperatures and proportions of solvent may vary from those mentioned above. In the case of dewaxed oils, or relatively less viscous oils, lower extraction temperatures may be employed. The extraction of the oil with the selective solvent may be carried out in either a continuous or stage countercurrent operation.

Extraction by the batch method of operation may also be employed.

Obviously, many modifications and variations of the invention, as hereinbefore set forth, may be made without departing from the spirit and scope thereof, but only such limitations should be imposed as are indicated in the appended claims.

I claim:

1. In the process of refining mineral lubricating oil with a selective solvent to produce therefrom a lubricating oil of high viscosity index, the method which comprises extracting the oil with a selective solvent to remove low viscosity index constituents as an extract phase and produce a raffinate phase comprising high viscosity index oil and retaining some extract phase, removing the raffinate phase, centrifuging the raffinate phase to remove retained extract phase material, and washing the centrifuged raffinate phase with a liquid having the solvent characteristics of methyl ethyl ketone to remove remaining retained material.

2. In the process of refining mineral lubricating oil with a selective solvent to produce therefrom a lubricating oil of high viscosity index, the method which comprises extracting the oil with a selective solvent to remove low viscosity index constituents as an extract phase and produce a raffinate phase comprising high viscosity index oil and retaining some extract phase, removing the raffinate phase, centrifuging the raffinate phase to remove retained extract phase material, washing the centrifuged raffinate phase with a liquid having the solvent characteristics of methyl ethyl ketone to remove remaining retained material, removing the wash solvent containing dissolved matter, separating the solvent from the dissolved material and returning the said material to the extraction zone. 40

3. In the process of refining mineral lubricating oil with a selective solvent to produce therefrom a lubricating oil of high viscosity index, the method which comprises extracting the oil with a solvent comprising furfural, in an extraction zone 45 at a temperature of around 200° F., forming an extract phase comprising low viscosity index constituents of the oil dissolved in the solvent, and a raffinate phase comprising high viscosity index constituents of the oil and retaining some extract phase, separating the two phases, cooling the raffinate phase to a temperature below the extraction temperature, centrifuging the cooled raffinate phase to separate retained extract phase material, and washing the centrifuged raffinate phase with a liquid having the solvent characteristics of methyl ethyl ketone to remove remaining retained material. 50 55

4. In the process of refining mineral lubricating oil with a selective solvent to produce therefrom a lubricating oil of high viscosity index, the method which comprises extracting the oil with a solvent comprising furfural, in an extraction zone at a temperature of around 150-250° F., forming an extract phase comprising low viscosity index constituents of the oil dissolved in the solvent, and a raffinate phase comprising high viscosity index constituents of the oil and retaining some extract phase, separating the two phases, cooling the raffinate phase to a temperature below the extraction temperature, centrifuging the cooled raffinate phase to separate retained extract phase material, returning the separated material to the extraction zone, washing the centrifuged raffinate phase with a liquid having

ing the solvent characteristics of methyl ethyl ketone to remove remaining retained material, removing the wash solvent and dissolved material, separating the solvent from the dissolved material, and returning said dissolved material to the extraction zone.

5. In the process of refining wax-bearing mineral lubricating oil with a selective solvent to produce therefrom a lubricating oil of high viscosity index, the method which comprises extracting the oil with furfural at a temperature substantially above atmospheric temperature to remove low viscosity index constituents as an extract phase and produce a raffinate phase comprising high viscosity index constituents and retaining some extract phase, removing the raffinate phase, cooling the raffinate phase to a temperature below the extraction temperature to separate retained extract phase material, removing the thus separated material, washing the remaining raffinate phase with a solvent having the solvent characteristics of methyl ethyl ketone to remove remaining retained material, and dewaxing the washed raffinate phase.

25. 6. In the process of refining wax-bearing mineral lubricating oil with a selective solvent to produce therefrom a lubricating oil of high viscosity index and low pour test, the method which comprises extracting the oil with a solvent comprising furfural, at a temperature of 150-250° F., while at such temperature forming an extract phase comprising dissolved oil of low viscosity index and retaining some oil of intermediate character as regards viscosity index, and a raffinate phase comprising high viscosity index constituents of the oil and retaining some of the extract phase, separating the two phases, cooling the raffinate phase to a temperature just above that at which it solidifies, centrifuging the cooled raffinate phase to remove retained extract phase material, washing the centrifuged raffinate phase with a solvent having the solvent characteristics of methyl ethyl ketone to remove remaining retained extract phase material, removing the wash solvent and dissolved bodies, and dewaxing the washed raffinate phase.

7. In the process of refining wax-bearing mineral lubricating oil with a selective solvent to produce therefrom a lubricating oil of high viscosity index and low pour test, the method which comprises extracting the oil with a solvent having at a temperature of 150° F. and above the essential selective action of furfural as between constituents of the oil of differing viscosity indices, forming an extract phase containing low viscosity index constituents dissolved in the solvent, and a raffinate phase comprising high viscosity index constituents including wax and retaining some extract phase, removing the raffinate phase, centrifuging the raffinate phase to remove retained extract phase material, washing the centrifuged raffinate phase with a liquid having the solvent characteristics of methyl ethyl ketone to remove remaining retained material, and dewaxing the washed raffinate phase in the presence of a chilled solvent mixture having selective action as between solid and high viscosity index hydrocarbons and having as a component part of such a chilled solvent mixture the wash solvent liquid retained by the raffinate phase.

8. In the process of refining wax-bearing mineral lubricating oil with a selective solvent to produce therefrom a lubricating oil of high viscosity index and low pour test, the method which comprises extracting the oil with a solvent com-

prising furfural in an extraction zone at a temperature around 200° F., forming an extract phase containing low viscosity index constituents dissolved in the solvent, and a raffinate phase comprising high viscosity index constituents including wax and retaining some extract phase, removing the raffinate phase, cooling the raffinate phase to a temperature below the extraction temperature, centrifuging the cooled raffinate phase to remove retained material, washing the centrifuged raffinate phase with a liquid having the solvent characteristics of methyl ethyl ketone, to remove remaining retained material, returning the retained material separated from the raffinate phase during the centrifuging and washing steps to the extraction zone, and dewaxing the washed raffinate phase in the presence of a chilled solvent mixture having selective action as between solid and high viscosity index hydrocarbons and having as a component part of such a chilled solvent mixture the wash solvent liquid retained by the raffinate phase.

9. In the process of refining mineral lubricating oil with a selective solvent to produce therefrom a lubricating oil of high viscosity index and low pour test, the method which comprises extracting the oil in an extraction zone at a temperature substantially above atmospheric with a solvent having at a temperature of 150° F. and above the essential selective action of furfural as between constituents of the oil of differing viscosity indices, forming an extract phase containing low viscosity index constituents dissolved in the solvent and retaining some oil of intermediate character as regards viscosity index constituents of the oil and a raffinate phase comprising high viscosity index constituents and retaining some of the extract phase, separating the two phases, separately cooling the two phases to separate retained material, removing the thus separated material, washing the raffinate phase with a solvent having the solvent characteristics of methyl ethyl ketone to remove remaining retained material and returning the retained materials separated from each phase to the extraction zone.

10. In the process of refining wax bearing mineral lubricating oil with a selective solvent to produce therefrom a lubricating oil of high viscosity index and low pour test, the method which comprises extracting the oil in an extraction zone at a temperature above atmospheric with a solvent having at a temperature of 150° F. and above the essential selective action of furfural as between constituents of the oil of differing viscosity indices, forming an extract phase containing low viscosity index constituents dissolved in the solvent and retaining some oil of intermediate character as regards viscosity index, and a raffinate phase comprising high viscosity index constituents of the oil and retaining some of the extract phase, separating the two phases, separately cooling the two phases to separate retained material, removing the thus separated material, washing the raffinate phase with a solvent having the solvent characteristics of methyl ethyl ketone to remove remaining retained material and returning the retained materials separated from each phase to the extraction zone, and dewaxing the raffinate phase in the presence of a chilled solvent mixture having selective action between solid and high viscosity index hydrocarbons and having as a component part of such chilled solvent mixture the wash solvent liquid retained by the washed raffinate phase.

11. In the process of refining wax bearing mineral lubricating oil with a selective solvent to produce therefrom a lubricating oil of high viscosity index and low pour test, the method which 5 comprises extracting the oil in an extraction zone with a solvent comprising furfural, at a temperature in the range of 150-250° F., while at such temperature forming an extract phase comprising dissolved oil of low viscosity index 10 and retaining some oil of intermediate character as regards viscosity index, and a raffinate phase comprising high viscosity index constituents of the oil and retaining some of the extract phase, separating the two phases, separately cooling the 15 two phases to a temperature substantially below the extraction temperature, centrifuging the cooled raffinate phase to remove retained extract phase material, settling the cooled extract phase to remove retained relatively high viscosity index oil, washing the centrifuged raffinate phase with a solvent having the solvent characteristics of methyl ethyl ketone adapted to remove remaining retained extract phase material, returning the bodies separated from the two 20 phases to the extraction zone, and dewaxing the 25 washed raffinate phase.
12. In the process of refining wax bearing mineral lubricating oil with a selective solvent to produce therefrom a lubricating oil of high viscosity index and low pour test, the method which 30 comprises extracting the oil with a solvent comprising furfural, at a temperature in the range of 150-250° F., while at such temperature forming an extract phase comprising dissolved oil of low viscosity index and retaining some oil of intermediate character as regards viscosity index, and a raffinate phase comprising high viscosity index constituents of the oil and retaining some 35 of the extract phase, separating the two phases, cooling the raffinate phase to a temperature substantially below the extraction temperature, centrifuging the cooled raffinate phase to remove retained extract phase material, washing the centrifuged raffinate phase with methyl ethyl ketone to remove remaining impurities, mixing 40 with the washed raffinate phase further methyl ethyl ketone together with a modifying solvent of the character of benzol, in proportions such that the solvent mixture has selective action as between solid and liquid hydrocarbons at temperatures of the order of 0° F., chilling the resulting mixture to precipitate the wax and separating the thus precipitated wax and removing the solvent liquids from the dewaxed oil.
- 40

FRANCIS X. GOVERS.